

July 23, 1935.

A. C. SIMMONS

2,008,879

METHOD OF COATING ARTICLES

Filed Nov. 11, 1933

FIG. 1



FIG. 2



INVENTOR  
A. C. SIMMONS  
BY H. G. Whitehorn  
ATTORNEY

## UNITED STATES PATENT OFFICE

2,008,879

## METHOD OF COATING ARTICLES

Andrew C. Simmons, Peoria, Ill., assignor to  
 Western Electric Company, Incorporated, New  
 York, N. Y., a corporation of New York

Application November 11, 1933, Serial No. 697,585

9 Claims. (Cl. 91—70.2)

This invention relates to a method of coating articles, and more particularly to a method of hot galvanizing articles.

It is common practice in galvanizing articles to provide a molten bath of zinc covered with a suitable fluxing material to prevent the zinc from oxidizing. The articles to be galvanized, particularly in the case of small articles, are placed in a perforated basket and dipped in the zinc bath and before removing the basket from the bath the layer of flux, which may be several inches thick, must be skimmed to one side to prevent it from coming into contact with and thereby contaminating the galvanized articles as they are removed from the bath. This method also leaves such a heavy coating of zinc on the articles that usually, particularly in the case of screw threaded articles and other articles requiring close tolerance limits, other methods must be resorted to after the articles have been dipped to remove the excess zinc therefrom in order to provide a smooth uniform coating and bring the articles within the desired tolerance limits.

It has been attempted to overcome the above mentioned difficulties by adding various metals to the zinc bath to increase the fluidity thereof, some of the metals added being aluminum, tin, antimony, bismuth, or a combination of these metals. When certain of these metals are added, particularly aluminum, it becomes very difficult to maintain the proper immersion flux on the surface of the bath, and the alloy becomes unstable when the surface is exposed to the reducing action of the flux. The addition of aluminum also retards the galvanizing operation because the zinc aluminum alloy does not adhere to ferrous metals as readily as unalloyed zinc, thereby prolonging the time required to apply a given thickness of coating.

An object of this invention is to provide an improved method of coating articles in an expeditious and economical manner to provide a smooth, uniform coating.

In accordance with the general features of the invention, one embodiment of an apparatus by means of which the method may be practiced, as applied to the galvanizing of small articles, comprises a molten zinc bath covered with a fluxing material and a molten zinc aluminum alloy bath adjacent thereto, the alloy bath being maintained sufficiently full so that the fluid level thereof will be located above the level of the zinc bath and arranged to overflow into the zinc bath when the alloy is displaced upon the dipping of articles therein. In practicing the method a basket of

articles to be galvanized is dipped into the zinc bath, where they acquire a heavy coating, and then withdrawn without skimming the flux from the surface of the bath and immediately dipped into the zinc aluminum bath adjacent the point of overflow which serves to wash the articles of any excess zinc carried thereon from the zinc bath, due to the greater fluidity of the alloy bath, and gives the articles a smooth, uniform coating. During the dipping of the zinc coated articles into the zinc aluminum bath the flux carried from the zinc bath floats to the surface of the alloy bath and the level of the latter bath is sufficiently raised so that the flux carried thereinto is washed back into the zinc bath. Before removing the basket of articles from the alloy bath it is moved horizontally while immersed therein to another position farther away from the point of overflow to insure that none of the flux will come into contact with the alloy washed articles as they are withdrawn.

Other objects and advantages of this invention will more fully appear from the following detailed description taken in connection with the accompanying drawing which illustrates one embodiment of an apparatus by means of which the method may be practiced, in which

Fig. 1 is a diagrammatic side view, partly in section, of an apparatus used in practicing the method of this invention, and

Fig. 2 is a vertical section taken on the line 2—2 thereof.

Referring to the drawing, the numeral 10 indicates a galvanizing receptacle or tank containing a bath 11 of molten zinc, the level of which is indicated at 12. The bath of zinc 11 is kept molten and at a desired temperature by any suitable heat applying means (not shown). Any suitable galvanizing flux, such as sal-ammoniac, indicated at 13, and which is several inches thick, can be used on the surface of the zinc bath. Inserted in and adjacent one end of the tank 10 is a receptacle or tank 14 having upper side flanges 15 supported upon similar flanges 16 of the tank 10 with its side, end, and bottom walls spaced from the walls of the tank 10. The left end wall of the tank 14 is cut down so that its upper edge 17 is below the upper edge of the right end wall of the tank 14. The level 12 of the zinc bath 11 is kept suitably below the upper edge 17 of the left end wall of the tank 14 so that the molten zinc will not flow into the tank 14.

A bath 18 comprising a sufficient volume of molten zinc aluminum alloy is maintained in the

tank 14 so that when the alloy is displaced by the immersion therein of the articles to be treated to be presently described, its fluid level, indicated at 19, will rise and overflow in the plane of 5 the upper edge 17 of the left end wall and wash the flux carried thereinto with the articles into the zinc bath 11. The range of aluminum in the alloy bath 18 is not at all critical but in practice from .2% to 1% of aluminum is added, which 10 makes the bath more fluid for a purpose made apparent hereinafter. While in the embodiment of the apparatus illustrated the alloy bath 18 is kept molten by the heat transmitted from the molten zinc bath 11 which surrounds the 15 tank 14 individual heating means could be used for each bath and thus eliminate the attack of zinc on the outside surface of the tank 14, which is of iron.

In practicing the invention, the baths 11 and 20 18 are first prepared in the manner described hereinbefore and the articles to be galvanized are placed in a perforated basket 20 which is then submerged or dipped into the zinc bath 11 by suitable handling means, fragmentarily indicated at 21, as shown at the left end of the tank 10 (Fig. 1). The basket 20 is left submerged in the bath 11 for a suitable period of time and then withdrawn without skimming the flux 13 from the surface of the bath, with the result that a 25 quantity of flux will be left deposited on the upper layer of articles in the basket. Immediately upon being withdrawn from the bath 11, by the means 21, the basket 20 of zinc coated articles is moved to the right and lowered to a position 30 indicated at 22 into the zinc aluminum bath 18 to wash the articles of any excess zinc carried thereon from the zinc bath 11. In the dipping of the coated articles in the bath 18 which is sufficiently full, as hereinbefore described, to 35 cause its fluid level 19 to rise and overflow in the plane of the upper edge 17 of the left wall of the tank 14, the flux 13 carried along by the basket 20 from the zinc bath 11 floats to the surface of the bath 18. The immersion of the coated articles in the alloy bath 18 raises the level 40 19 thereof sufficiently to cause the flux 13 thereon to be washed back into the zinc bath 11. Although the surface of the bath 18 is not at all 45 times clear of the flux 13, since all of it may not be washed over the edge 17 at each dipping of a basket 20 of coated articles, it will at least float over towards the edge 17 or the overflow point, as indicated at 23. After being submerged 50 for a suitable period of time in the alloy bath 18 at the position 22, the basket 20 of treated articles is moved horizontally, while still immersed in the bath, to a position indicated at 24 55 farther away from the point of overflow where the surface of the alloy bath is free of the flux 13, or other foreign matter, thereby insuring that none of the flux, or foreign matter, which may still remain on the surface of the bath adjacent the edge 17 of the tank 14 will come into 60 contact with and contaminate the articles which have been treated and washed in the alloy bath 65 when they are withdrawn therefrom. The basket 20 of galvanized articles is then withdrawn from the alloy bath 18 at the position 24, which step completes the method of this invention.

70 It is understood that although the excess zinc washed from the articles in the alloy bath 18 helps to maintain the latter bath full to overflowing when the articles are immersed therein so that it will be effective to wash the flux into the zinc bath 11 in the manner above described,

it may be necessary at times to make suitable additions of zinc and aluminum to the alloy bath 18, particularly of aluminum, since some of the aluminum is removed by the flux washed into the bath 11.

5 The aluminum in the alloy bath 18 is a strong deoxidizing agent and tends to make the zinc quite fluid so that there will be only a small excess of zinc, if any, on the objects when they are withdrawn from the bath 18. Thus a very 10 smooth and more uniform coating is imparted to articles which have immediately preceding been given a galvanizing coating, and thereby permitting, particularly in the case of screw threaded articles and other articles, the bringing of them within the desired tolerance limits. It will be understood that due to the deoxidizing effect of the aluminum in the alloy bath, it is not necessary to have this bath covered by a 15 flux.

20 It will be obvious that in the method of galvanizing objects hereinbefore described wherein a combination of a zinc bath and a zinc aluminum alloy bath is employed articles may be expeditiously and economically treated as compared to the use of a single zinc aluminum alloy bath, since the latter type of bath requires a longer time for a given thickness of zinc, due to the presence of aluminum therein.

Although the invention is illustrated and described as applied to the galvanizing of comparatively small articles carried in a basket or other type of carrier, it should be understood that the same is applicable to large articles with or without the employment of a carrier which is immersed in the baths along with the article to be treated. Also the invention is not limited to the treating of articles with zinc and zinc aluminum alloys, but other ingredients may be substituted for aluminum. Furthermore, although a specific 40 form of apparatus for practicing the steps of the method has been disclosed as exemplifying the embodiment of the invention, it is understood that other forms of apparatus might be used, and the invention is limited only by the spirit and 45 scope of the appended claims. The principle of the invention is also applicable to any case where it is desirable to immerse articles first in a bath having a covering of flux and then into a bath requiring no flux, assuming, of course, that the 50 two baths are of such materials that a small portion of each may be safely allowed to mix with the other bath.

55 What is claimed is:

1. A method of coating an article which comprises first passing the article through flux floating upon a bath of molten metal and immersing it in said bath, withdrawing the coated article therefrom and moving it through the flux, immersing it in a second bath of molten metal which 60 is sufficiently full to cause flux carried thereinto with the article and washed from the article to be washed from the second bath in an overflow thereof when the article is immersed therein, and then withdrawing the article from the second 65 bath.

70 2. A method of coating an article which comprises first passing the article through flux floating upon a bath of molten metal and immersing it in said bath, withdrawing the coated article therefrom and moving it through the flux, immersing it in a second bath of molten metal of greater fluidity than the first bath which is sufficiently full to cause flux carried thereinto with the article and washed from the article to be 75

washed from the second bath in an overflow thereof when the article is immersed therein, and then withdrawing the article from the second bath.

- 5 3. A method of coating an article which comprises first passing the article through a layer of flux floating upon a bath of molten metal and immersing it in said bath of molten metal, withdrawing the coated article therefrom and through 10 the layer of flux, immersing it in a second bath of molten metal which is sufficiently full to cause flux carried thereinto with the article and washed from the article to be washed from the second bath in an overflow thereof when the article is 15 immersed therein, moving the article while still immersed to a position removed from its initial position of immersion, and then withdrawing the article from the second bath.
4. A method of galvanizing an article which 20 comprises first immersing the article in a bath of molten zinc having flux floating upon its surface, withdrawing the zinc coated article therefrom and through the flux, immersing it in a bath of molten zinc aluminum alloy which is sufficiently full to cause flux carried thereinto with the article and washed from the article to be 25 washed from the alloy bath in an overflow thereof when the article is immersed therein, and then withdrawing the alloy treated zinc coated article 30 from the alloy bath.
5. A method of galvanizing an article which comprises first immersing the article in a bath of molten zinc having a layer of flux floating upon its surface, withdrawing the zinc coated article 35 therefrom and through the flux, immersing it in a bath of molten zinc aluminum alloy which is sufficiently full to cause flux carried thereinto with the article and washed from the article to be washed from the alloy bath into the zinc bath 40 in an overflow of the alloy bath when the article is immersed therein, moving the article while still immersed to a position removed from its initial position of immersion, and then withdrawing the alloy treated zinc coated article from the alloy 45 bath.
6. A method of galvanizing articles in a bath of molten zinc having a flux thereon and a bath of
- molten zinc aluminum alloy which comprises immersing the articles in the zinc bath, withdrawing the articles from the zinc bath and through the flux, immersing the articles in the second bath to cause overflowing thereof to wash the flux removed from the articles from the second bath, and then withdrawing the articles from the second bath. 5
7. A method of galvanizing articles in a bath of molten zinc having a flux thereon and a bath of molten zinc aluminum alloy which comprises immersing the articles in the zinc bath, withdrawing the articles from the zinc bath and through the flux, immersing the articles in the second bath adjacent an end thereof to cause 10 overflowing of the second bath to wash the flux removed from the articles over the end of the second bath, and then withdrawing the articles from the second bath. 15
8. A method of galvanizing articles in a bath of molten zinc having a flux thereon and a bath of molten zinc aluminum alloy which comprises immersing the articles in the zinc bath, withdrawing the articles from the zinc bath and through the flux, immersing the articles in the second bath adjacent an end thereof to cause 20 overflowing of the second bath to wash the flux removed from the articles over the end of the second bath and into the zinc bath, moving the articles while still immersed in the second bath to a position removed from their initial 25 position of immersion, and then withdrawing the articles from the second bath. 30
9. A method of galvanizing articles in a bath of molten zinc having a flux thereon and a bath of molten zinc aluminum alloy which comprises immersing the articles in the zinc bath, withdrawing the articles from the zinc bath and through the flux, immersing the articles in the second bath to cause overflowing thereof to wash 35 the flux removed from the articles from the second bath, moving the articles while still immersed in the second bath to a position removed from their initial position of immersion, and then withdrawing the articles from the second bath. 40
- 45

ANDREW C. SIMMONS.